# EUROPEAN PATENT SPECIFICATION

(11) **EP 3 559 293 B1**
(45) Date of publication and mention of the grant of the patent: **20.08.2025**
(21) Application number: 17882929.7
(22) Date of filing: 28.11.2017
(51) Int. Cl.: C22C 21/10, B22D 11/00

(54) **HIGH ZINC ALUMINUM ALLOY PRODUCTS**
PRODUKTE AUS ZINKREICHER ALUMINIUMLEGIERUNG
PRODUITS D'ALLIAGE D'ALUMINIUM À TENEUR ÉLEVÉE EN ZINC

(30) Priority: 21.12.2016 US 201662437489 P
(43) Date of publication of application: 30.10.2019
(73) Proprietor: Arconic Technologies LLC, Pittsburgh, PA 15212 (US)
(72) Inventor: UNAL, Ali, Export, PA 15632 (US); NEWMAN, John, Monroeville, PA 15146 (US); TOMES, David, San Antonio, TX 78261 (US); WYATT-MAIR, Gavin, Lafayette, CA 94549 (US)
(74) Representative: Forresters IP LLP
(86) International application number: PCT/US2017/063481
(87) International publication number: WO 2018/118350

(56) References cited:
- WO-A2-2012/033939
- US-A- 3 791 880
- US-A- 5 135 713
- US-A1- 2002 121 319
- US-A1- 2002 153 123
- US-A1- 2005 269 000
- US-A1- 2015 064 058
- US-A1- 2015 064 058
- YUN-SOO LEE ET AL: "Recrystallization behavior of cold rolled Al-Zn-Mg-Cu fabricated by twin roll casting", TRANSACTIONS OF NONFERROUS METALS SOCIETY OF CHINA : ENGLISH EDITION = ZHONGGUO-YOUSE-JINSHU-XUEBAO, vol. 24, no. 7, 21 August 2014 (2014-08-21), AMSTERDAM, NL, pages 2226 - 2231, XP055680602, ISSN: 1003-6326, DOI: 10.1016/S1003-6326(14)63337-9
- SU X ET AL: "Abatement of segregation with the electro and static magnetic field during twin-roll casting of 7075 alloy sheet", MATERIALS SCIENCE AND ENGINEERING: A, vol. 599, 27 January 2014 (2014-01-27), pages 279 - 285, XP028628485, ISSN: 0921-5093, DOI: 10.1016/J.MSEA.2014.01.042

## Description

### BACKGROUND OF INVENTION

Casting aluminum alloys to form cast aluminum alloy products is known. US 2015/064058 discloses a method of manufacturing an aluminum-zinc-based alloy sheet using twin-roll casting.

### TECHNICAL FIELD

The present invention relates to cast aluminum alloy products, and products derived therefrom.

### BRIEF SUMMARY OF INVENTION

The present invention is a cast product as defined in claim 1.

In one or more embodiments detailed herein, the aluminum alloy strip comprises 6 wt. % to 28 wt. % zinc. In one or more embodiments detailed herein, the aluminum alloy strip comprises 8 wt. % to 28 wt. % zinc. In one or more embodiments detailed herein, the aluminum alloy strip comprises 10 wt. % to 28 wt. % zinc. In one or more embodiments detailed herein, the aluminum alloy strip comprises 4 wt. % to 15 wt. % zinc. In one or more embodiments detailed herein, the aluminum alloy strip comprises 6 wt. % to 12 wt. % zinc. In one or more embodiments detailed herein, the aluminum alloy strip comprises 4 wt. % to 10 wt. % zinc. In one or more embodiments detailed herein, the aluminum alloy strip comprises 4 wt. % to 8 wt. % zinc.

In one or more embodiments detailed herein, the variation of the zinc weight percent is 12% or less between the surface and the thickness center of the aluminum alloy strip.

In one or more embodiments detailed herein, the aluminum alloy strip comprises: (i) 4 wt. % to 28 wt. % zinc; (ii) 1 wt. % to 3 wt. % copper; and (iii) 1 wt. % to 3 wt. % magnesium.

In one or more embodiments detailed herein, the aluminum alloy strip comprises 4 wt. % to 15 wt. % zinc. In one or more embodiments detailed herein, the aluminum alloy strip comprises 4 wt. % to 12 wt. % zinc. In one or more embodiments detailed herein, the aluminum alloy strip comprises 4 wt. % to 10 wt. % zinc.

In one or more embodiments detailed herein, the aluminum alloy strip comprises 1 wt. % to 2.5 wt. % copper. In one or more embodiments detailed herein, the aluminum alloy strip comprises 1 wt. % to 2.0 wt. % copper. In one or more embodiments detailed herein, the aluminum alloy strip comprises 1 wt. % to 1.5 wt. % copper.

In one or more embodiments detailed herein, the aluminum alloy strip comprises 1 wt. % to 2.5 wt. % magnesium. In one or more embodiments detailed herein, the aluminum alloy strip comprises 1 wt. % to 2.0 wt. % magnesium. In one or more embodiments detailed herein, the aluminum alloy strip comprises 1 wt. % to 1.5 wt. % magnesium.

In one or more embodiments detailed herein, the aluminum alloy strip comprises: 4 wt. % to 28 wt. % zinc and 1 wt. % to 3 wt. % copper..

### BRIEF DESCRIPTION OF THE DRAWINGS

FIG. 1 is a schematic of a non-limiting method of making the cast product;
FIG. 2 is an enlarged cross-sectional schematic of the molten metal delivery tip and rolls shown in FIG. 1;
FIG. 3 shows the variation in zinc weight percentage from surface to a thickness depth of 3,000 micrometers in a cast product;
FIG. 4 shows the variation in zinc weight percentage from surface to a thickness depth of 3,000 micrometers in a cast product;
FIG. 5 shows the variation in zinc weight percentage from surface to a thickness depth of 3,000 micrometers in a cast product;
FIG. 6 shows the variation in zinc weight percentage from surface to a thickness depth of 3,000 micrometers in a cast product;
FIG. 7 shows the variation in zinc weight percentage from surface to a thickness depth of 3,000 micrometers in a cast product;
FIG. 8 shows the variation in zinc weight percentage from surface to a thickness depth of 3,000 micrometers in a cast product;
FIG. 9 shows the variation in zinc weight percentage from surface to a thickness depth of 3,000 micrometers in a cast product;
FIG. 10 shows the variation in zinc weight percentage from surface to a thickness depth of 3,000 micrometers in a cast product;
FIG. 11 shows the variation in zinc weight percentage through depth of a prior art ingot cast by direct chill casting;
FIG. 12 shows the variation in zinc weight percentage through depth of a prior art cast product;
FIG. 13 shows the weight percentages of zinc, magnesium and copper across grains from the surface to 200 micrometers thickness depth in a cast product according to an embodiment of the present invention.
FIG. 14 shows the weight percentages of the zinc, magnesium and copper across grains through thickness depth for a direct chill cast prior art product;
FIG. 15 shows the structure of a cast product according to an embodiment of the present invention;
FIG. 16 shows the structure of a cast product according to an embodiment of the present invention; and
FIG. 17 shows the structure of a cast product according to an embodiment of the present invention.

The figures constitute a part of this specification and include illustrative embodiments of the present invention and illustrate various objects and features thereof. Further, the figures are not necessarily to scale, some features may be exaggerated to show details of particular components. In addition, any measurements, specifications and the like shown in the figures are intended to be illustrative, and not restrictive. Therefore, specific structural and functional details disclosed herein are not to be interpreted as limiting, but merely as a representative basis for teaching one skilled in the art to variously employ the present invention.

The present invention will be further explained with reference to the attached drawings, wherein like structures are referred to by like numerals throughout the several views. The drawings shown are not necessarily to scale, with emphasis instead generally being placed upon illustrating the principles of the present invention. Further, some features may be exaggerated to show details of particular components.

### DETAILED DESCRIPTION OF THE INVENTION

Among those benefits and improvements that have been disclosed, other objects and advantages of this invention will become apparent from the following description taken in conjunction with the accompanying figures. Detailed embodiments of the present invention are disclosed herein; however, it is to be understood that the disclosed embodiments are merely illustrative of the invention that may be embodied in various forms. In addition, each of the examples given in connection with the various embodiments of the invention are intended to be illustrative, and not restrictive.

Throughout the specification and claims, the following terms take the meanings explicitly associated herein, unless the context clearly dictates otherwise. The phrases "in one embodiment" and "in some embodiments" as used herein do not necessarily refer to the same embodiment(s), though they may. Furthermore, the phrases "in another embodiment" and "in some other embodiments" as used herein do not necessarily refer to a different embodiment, although they may. Thus, as described below, various embodiments of the invention may be readily combined, without departing from the scope of the claims.

In addition, as used herein, the term "or" is an inclusive "or" operator, and is equivalent to the term "and/or," unless the context clearly dictates otherwise. The term "based on" is not exclusive and allows for being based on additional factors not described, unless the context clearly dictates otherwise. In addition, throughout the specification, the meaning of "a," "an," and "the" include plural references. The meaning of "in" includes "in" and "on."

As used herein, the term "at least one of A, B, or C" and the like, means "only A", "only B", "only C", or "any combination of A, B, and C."

The present invention is defined in claim 1.

In one or more embodiments detailed herein, the aluminum alloy strip comprises 6 wt. % to 28 wt. % zinc. In one or more embodiments detailed herein, the aluminum alloy strip comprises 8 wt. % to 28 wt. % zinc. In one or more embodiments detailed herein, the aluminum alloy strip comprises 10 wt. % to 28 wt. % zinc. In one or more embodiments detailed herein, the aluminum alloy strip comprises 4 wt. % to 15 wt. % zinc. In one or more embodiments detailed herein, the aluminum alloy strip comprises 6 wt. % to 12 wt. % zinc. In one or more embodiments detailed herein, the aluminum alloy strip comprises 4 wt. % to 10 wt. % zinc. In one or more embodiments detailed herein, the aluminum alloy strip comprises 4 wt. % to 8 wt. % zinc.

In one or more embodiments detailed herein, the variation of the zinc weight percent is 12% or less between the surface and the thickness center of the aluminum alloy strip.

In one or more embodiments detailed herein, the aluminum alloy strip comprises: (i) 4 wt. % to 28 wt. % zinc; (ii) 1 wt. % to 3 wt. % copper; and (iii) 1 wt. % to 3 wt. % magnesium.

In one or more embodiments detailed herein, the aluminum alloy strip comprises 4 wt. % to 15 wt. % zinc. In one or more embodiments detailed herein, the aluminum alloy strip comprises 4 wt. % to 12 wt. % zinc. In one or more embodiments detailed herein, the aluminum alloy strip comprises 4 wt. % to 10 wt. % zinc.

In one or more embodiments detailed herein, the aluminum alloy strip comprises 1 wt. % to 2.5 wt. % copper. In one or more embodiments detailed herein, the aluminum alloy strip comprises 1 wt. % to 2.0 wt. % copper. In one or more embodiments detailed herein, the aluminum alloy strip comprises 1 wt. % to 1.5 wt. % copper.

In one or more embodiments detailed herein, the aluminum alloy strip comprises 1 wt. % to 2.5 wt. % magnesium. In one or more embodiments detailed herein, the aluminum alloy strip comprises 1 wt. % to 2.0 wt. % magnesium. In one or more embodiments detailed herein, the aluminum alloy strip comprises 1 wt. % to 1.5 wt. % magnesium.

In one or more embodiments detailed herein, the aluminum alloy strip comprises: 4 wt. % to 28 wt. % zinc and 1 wt. % to 3 wt. % copper

As used herein, the term "aluminum alloy" means an aluminum metal with soluble elements either in the aluminum lattice or in a phase within aluminum. Elements are added to influence physical properties of the aluminum alloy and performance characteristics.

As used herein, the phrase "7xxx aluminum alloys" and the like means an aluminum alloy selected from 7xxx aluminum alloys registered with the Aluminum Association and unregistered variants of the same.

As used herein, the term "cast product" means a product that has been produced by a casting method such as continuous casting as detailed in U.S. Patent Nos. 6,672,368 and 7,125,612. In one or more embodiments detailed herein, the term "cast product" includes a product produced from the "cast product". In one or more embodiments, the term "cast product" includes a rolled product produced from the "cast product".

As used herein, the term "variation" of the weight percent of an alloying element in a specified thickness depth of half thickness (T/2) has units of "%" and is calculated according to the following equation:
(maximum weight percent of alloying element in the specified thickness depth - minimum weight percent of the alloying element in the specified thickness depth)/(mean weight percent of the alloying element in the specified thickness depth) * 100.

As used herein, the term "centerline segregation" means the enrichment or depletion of alloying elements in a central portion of an aluminum alloy strip. In embodiments, centerline segregation is determined based on a variation of the weight percent of an alloying element in a specified thickness depth of an aluminum alloy strip. In one or more embodiments detailed herein, centerline segregation is determined based on a variation of weight percent of an alloying element of greater than 15% between a surface and a thickness center of the aluminum alloy strip.

As used herein, the "weight percent of an alloying element" in a specified thickness depth is determined using the **"macro-segregation procedure"** detailed herein.

As used herein, the term "strip" may be of any suitable thickness, and is generally of sheet gauge (0.152 mm to 6.32 mm (0.006 inch to 0.249 inch)) or thin-plate gauge (6.35 mm to 10.1 mm (0.250 inch to 0.400 inch)), i.e., has a thickness in the range of from 0.152 mm to 10.1 mm (0.006 inch to 0.400 inch). In one embodiment, the strip has a thickness of at least 1.02 mm (0.040 inch). In one embodiment, the strip has a thickness of less than 8.13 mm (0.320 inch). In one or more embodiments detailed herein, the strip has a thickness of from 0.178 to 4.57 mm (0.0070 to 0.18 inches). In one or more embodiments detailed herein, the strip has a thickness of from 2.03 to 5.08 mm (0.08 to 0.2 inches).

As used herein, "surface" means a top surface or a bottom surface of the cast product.

As used herein, "thickness center" means a depth of half the total thickness of the cast product or half thickness (t/2).

In one or more embodiments detailed herein, the aluminum alloy strip may include at least one of 1 wt. % to 3 wt. % copper and 1 wt. % to 3 wt. % magnesium. In one or more embodiments detailed herein, the aluminum alloy may include 7xxx (zinc based) aluminum alloys.

In one or more embodiments detailed herein, the aluminum alloy strip has 4 wt. % to 27 wt. % zinc. In one or more embodiments detailed herein, the aluminum alloy strip has 4 wt. % to 25 wt. % zinc. In one or more embodiments detailed herein, the aluminum alloy strip has 4 wt. % to 22 wt. % zinc. In one or more embodiments detailed herein, the aluminum alloy strip has 4 wt. % to 20 wt. % zinc. In one or more embodiments detailed herein, the aluminum alloy strip has 4 wt. % to 18 wt. % zinc. In one or more embodiments detailed herein, the aluminum alloy strip has 4 wt. % to 15 wt. % zinc. In one or more embodiments detailed herein, the aluminum alloy strip has 4 wt. % to 13 wt. % zinc. In one or more embodiments detailed herein, the aluminum alloy strip has 4 wt. % to 11 wt. % zinc. In one or more embodiments detailed herein, the aluminum alloy strip has 4 wt. % to 10 wt. % zinc. In one or more embodiments detailed herein, the aluminum alloy strip has 4 wt. % to 9 wt. % zinc. In one or more embodiments detailed herein, the aluminum alloy strip has 4 wt. % to 8 wt. % zinc. In one or more embodiments detailed herein, the aluminum alloy strip has 4 wt. % to 7 wt. % zinc. In one or more embodiments detailed herein, the aluminum alloy strip has 4 wt. % to 6 wt. % zinc. In one or more embodiments detailed herein, the aluminum alloy strip has 4 wt. % to 5 wt. % zinc.

In one or more embodiments detailed herein, the aluminum alloy strip has 5 wt. % to 28 wt. % zinc. In one or more embodiments detailed herein, the aluminum alloy strip has 6 wt. % to 28 wt. % zinc. In one or more embodiments detailed herein, the aluminum alloy strip has 7 wt. % to 28 wt. % zinc. In one or more embodiments detailed herein, the aluminum alloy strip has 8 wt. % to 28 wt. % zinc. In one or more embodiments detailed herein, the aluminum alloy strip has 9 wt. % to 28 wt. % zinc. In one or more embodiments detailed herein, the aluminum alloy strip has 10 wt. % to 28 wt. % zinc. In one or more embodiments detailed herein, the aluminum alloy strip has 11 wt. % to 28 wt. % zinc. In one or more embodiments detailed herein, the aluminum alloy strip has 13 wt. % to 28 wt. % zinc. In one or more embodiments detailed herein, the aluminum alloy strip has 15 wt. % to 28 wt. % zinc. In one or more embodiments detailed herein, the aluminum alloy strip has 18 wt. % to 28 wt. % zinc. In one or more embodiments detailed herein, the aluminum alloy strip has 20 wt. % to 28 wt. % zinc. In one or more embodiments detailed herein, the aluminum alloy strip has 22 wt. % to 28 wt. % zinc.

In one or more embodiments detailed herein, the aluminum alloy strip has 5 wt. % to 27 wt. % zinc. In one or more embodiments detailed herein, the aluminum alloy strip has 7 wt. % to 25 wt. % zinc. In one or more embodiments detailed herein, the aluminum alloy strip has 8 wt. % to 23 wt. % zinc. In one or more embodiments detailed herein, the aluminum alloy strip has 9 wt. % to 20 wt. % zinc. In one or more embodiments detailed herein, the aluminum alloy strip has 10 wt. % to 18 wt. % zinc. In one or more embodiments detailed herein, the aluminum alloy strip has 12 wt. % to 15 wt. % zinc.

In one or more embodiments detailed herein, the aluminum alloy strip has 1 wt. % to 2.8 wt. % copper. In one or more embodiments detailed herein, the aluminum alloy strip has 1 wt. % to 2.6 wt. % copper. In one or more embodiments detailed herein, the aluminum alloy strip has 1 wt. % to 2.4 wt. % copper. In one or more embodiments detailed herein, the aluminum alloy strip has 1 wt. % to 2.2 wt. % copper. In one or more embodiments detailed herein, the aluminum alloy strip has 1 wt. % to 2.0 wt. % copper. In one or more embodiments detailed herein, the aluminum alloy strip has 1 wt. % to 1.8 wt. % copper. In one or more embodiments detailed herein, the aluminum alloy strip has 1 wt. % to 1.6 wt. % copper. In one or more embodiments detailed herein, the aluminum alloy strip has 1 wt. % to 1.4 wt. % copper. In one or more embodiments detailed herein, the aluminum alloy strip has 1 wt. % to 1.2 wt. % copper.

In one or more embodiments detailed herein, the aluminum alloy strip has 1.2 wt. % to 3 wt. % copper. In one or more embodiments detailed herein, the aluminum alloy strip has 1.4 wt. % to 3 wt. % copper. In one or more embodiments detailed herein, the aluminum alloy strip has 1.6 wt. % to 3 wt. % copper. In one or more embodiments detailed herein, the aluminum alloy strip has 1.8 wt. % to 3 wt. % copper. In one or more embodiments detailed herein, the aluminum alloy strip has 2.0 wt. % to 3 wt. % copper. In one or more embodiments detailed herein, the aluminum alloy strip has 2.2 wt. % to 3 wt. % copper. In one or more embodiments detailed herein, the aluminum alloy strip has 2.4 wt. % to 3 wt. % copper. In one or more embodiments detailed herein, the aluminum alloy strip has 2.6 wt. % to 3 wt. % copper. In one or more embodiments detailed herein, the aluminum alloy strip has 2.8 wt. % to 3 wt. % copper.

In one or more embodiments detailed herein, the aluminum alloy strip has 1.2 wt. % to 2.8 wt. % copper. In one or more embodiments detailed herein, the aluminum alloy strip has 1.4 wt. % to 2.6 wt. % copper. In one or more embodiments detailed herein, the aluminum alloy strip has 1.6 wt. % to 2.4 wt. % copper. In one or more embodiments detailed herein, the aluminum alloy strip has 1.8 wt. % to 2.2 wt. % copper.

In one or more embodiments detailed herein, the aluminum alloy strip has 1 wt. % to 2.8 wt. % magnesium. In one or more embodiments detailed herein, the aluminum alloy strip has 1 wt. % to 2.6 wt. % magnesium. In one or more embodiments detailed herein, the aluminum alloy strip has 1 wt. % to 2.4 wt. % magnesium. In one or more embodiments detailed herein, the aluminum alloy strip has 1 wt. % to 2.2 wt. % magnesium. In one or more embodiments detailed herein, the aluminum alloy strip has 1 wt. % to 2.0 wt. % magnesium. In one or more embodiments detailed herein, the aluminum alloy strip has 1 wt. % to 1.8 wt. % magnesium. In one or more embodiments detailed herein, the aluminum alloy strip has 1 wt. % to 1.6 wt. % magnesium. In one or more embodiments detailed herein, the aluminum alloy strip has 1 wt. % to 1.4 wt. % magnesium. In one or more embodiments detailed herein, the aluminum alloy strip has 1 wt. % to 1.2 wt. % magnesium.

In one or more embodiments detailed herein, the aluminum alloy strip has 1.2 wt. % to 3 wt. % magnesium. In one or more embodiments detailed herein, the aluminum alloy strip has 1.4 wt. % to 3 wt. % magnesium. In one or more embodiments detailed herein, the aluminum alloy strip has 1.6 wt. % to 3 wt. % magnesium. In one or more embodiments detailed herein, the aluminum alloy strip has 1.8 wt. % to 3 wt. % magnesium. In one or more embodiments detailed herein, the aluminum alloy strip has 2.0 wt. % to 3 wt. % magnesium. In one or more embodiments detailed herein, the aluminum alloy strip has 2.2 wt. % to 3 wt. % magnesium. In one or more embodiments detailed herein, the aluminum alloy strip has 2.4 wt. % to 3 wt. % magnesium. In one or more embodiments detailed herein, the aluminum alloy strip has 2.6 wt. % to 3 wt. % magnesium. In one or more embodiments detailed herein, the aluminum alloy strip has 2.8 wt. % to 3 wt. % magnesium.

In one or more embodiments detailed herein, the aluminum alloy strip has 1.2 wt. % to 2.8 wt. % magnesium. In one or more embodiments detailed herein, the aluminum alloy strip has 1.4 wt. % to 2.6 wt. % magnesium. In one or more embodiments detailed herein, the aluminum alloy strip has 1.6 wt. % to 2.4 wt. % magnesium. In one or more embodiments detailed herein, the aluminum alloy strip has 1.8 wt. % to 2.2 wt. % magnesium.

In one or more embodiments detailed herein, the aluminum alloy strip has 0.1 wt. % to 1.0 wt. % manganese. In one or more embodiments detailed herein, the aluminum alloy strip has 0.2 wt. % to 1.0 wt. % manganese. In one or more embodiments detailed herein, the aluminum alloy strip has 0.4 wt. % to 1.0 wt. % manganese. In one or more embodiments detailed herein, the aluminum alloy strip has 0.6 wt. % to 1.0 wt. % manganese. In one or more embodiments detailed herein, the aluminum alloy strip has 0.8 wt. % to 1.0 wt. % manganese.

In one or more embodiments detailed herein, the aluminum alloy strip has 0.1 wt. % to 0.8 wt. % manganese. In one or more embodiments detailed herein, the aluminum alloy strip has 0.1 wt. % to 0.9 wt. % manganese. In one or more embodiments detailed herein, the aluminum alloy strip has 0.1 wt. % to 0.7 wt. % manganese. In one or more embodiments detailed herein, the aluminum alloy strip has 0.1 wt. % to 0.5 wt. % manganese. In one or more embodiments detailed herein, the aluminum alloy strip has 0.1 wt. % to 0.3 wt. % manganese.

In one or more embodiments detailed herein, the aluminum alloy strip has 0.05 wt. % to 0.3 wt. % chromium. In one or more embodiments detailed herein, the aluminum alloy strip has 0.1 wt. % to 0.3 wt. % chromium. In one or more embodiments detailed herein, the aluminum alloy strip has 0.15 wt. % to 0.3 wt. % chromium. In one or more embodiments detailed herein, the aluminum alloy strip has 0.2 wt. % to 0.3 wt. % chromium. In one or more embodiments detailed herein, the aluminum alloy strip has 0.25 wt. % to 0.3 wt. % chromium.

In one or more embodiments detailed herein, the aluminum alloy strip has 0.05 wt. % to 0.25 wt. % chromium. In one or more embodiments detailed herein, the aluminum alloy strip has 0.05 wt. % to 0.2 wt. % chromium. In one or more embodiments detailed herein, the aluminum alloy strip has 0.05 wt. % to 0.15 wt. % chromium. In one or more embodiments detailed herein, the aluminum alloy strip has 0.05 wt. % to 0.1 wt. % chromium. In one or more embodiments detailed herein, the aluminum alloy strip has 0.15 wt. % to 0.25 wt. % chromium.

In one or more embodiments detailed herein, the aluminum alloy strip has 0.04 wt. % to 0.25 wt. % zirconium. In one or more embodiments detailed herein, the aluminum alloy strip has 0.04 wt. % to 0.2 wt. % zirconium. In one or more embodiments detailed herein, the aluminum alloy strip has 0.04 wt. % to 0.18 wt. % zirconium. In one or more embodiments detailed herein, the aluminum alloy strip has 0.04 wt. % to 0.15 wt. % zirconium. In one or more embodiments detailed herein, the aluminum alloy strip has 0.04 wt. % to 0.1 wt. % zirconium.

In one or more embodiments detailed herein, the aluminum alloy strip has 0.1 wt. % to 0.25 wt. % zirconium. In one or more embodiments detailed herein, the aluminum alloy strip has 0.15 wt. % to 0.25 wt. % zirconium. In one or more embodiments detailed herein, the aluminum alloy strip has 0.2 wt. % to 0.25 wt. % zirconium.

In one or more embodiments detailed herein, the aluminum alloy strip has 0.07 wt. % to 0.14 wt. % zirconium.

In one or more embodiments detailed herein, the aluminum alloy strip is free of at least one of copper, magnesium, manganese, chromium, or zirconium.

In one or more embodiments detailed herein, a variation of the zinc weight percent between a surface and a thickness center of the aluminum alloy strip is 14% or less. In one or more embodiments detailed herein, a variation of the zinc weight percent between a surface and a thickness center of the aluminum alloy strip is 13% or less. In one or more embodiments detailed herein, a variation of the zinc weight percent between a surface and a thickness center of the aluminum alloy strip is 12% or less. In one or more embodiments detailed herein, a variation of the zinc weight percent between a surface and a thickness center of the aluminum alloy strip is 11% or less. In one or more embodiments detailed herein, a variation of the zinc weight percent between a surface and a thickness center of the aluminum alloy strip is 10% or less. In one or more embodiments detailed herein, a variation of the zinc weight percent between a surface and a thickness center of the aluminum alloy strip is 9% or less. In one or more embodiments detailed herein, a variation of the zinc weight percent between a surface and a thickness center of the aluminum alloy strip is 8% or less. In one or more embodiments detailed herein, a variation of the zinc weight percent between a surface and a thickness center of the aluminum alloy strip is 7% or less. In one or more embodiments detailed herein, a variation of the zinc weight percent between a surface and a thickness center of the aluminum alloy strip is 6% or less. In one or more embodiments detailed herein, a variation of the zinc weight percent between a surface and a thickness center of the aluminum alloy strip is 5% or less. In one or more embodiments detailed herein, a variation of the zinc weight percent between a surface and a thickness center of the aluminum alloy strip is 4% or less. In one or more embodiments detailed herein, a variation of the zinc weight percent between a surface and a thickness center of the aluminum alloy strip is 3% or less. In one or more embodiments detailed herein, a variation of the zinc weight percent between a surface and a thickness center of the aluminum alloy strip is 2% or less.

In one or more embodiments detailed herein, a variation of the zinc weight percent between a surface and a thickness center of the aluminum alloy strip is 0.1% to 15%. In one or more embodiments detailed herein, a variation of the zinc weight percent between a surface and a thickness center of the aluminum alloy strip is 0.1% to 14%. In one or more embodiments detailed herein, a variation of the zinc weight percent between a surface and a thickness center of the aluminum alloy strip is 0.1% to 13%. In one or more embodiments detailed herein, a variation of the zinc weight percent between a surface and a thickness center of the aluminum alloy strip is 0.1% to 12%. In one or more embodiments detailed herein, a variation of the zinc weight percent between a surface and a thickness center of the aluminum alloy strip is 0.1% to 11%. In one or more embodiments detailed herein, a variation of the zinc weight percent between a surface and a thickness center of the aluminum alloy strip is 0.1% to 10%. In one or more embodiments detailed herein, a variation of the zinc weight percent between a surface and a thickness center of the aluminum alloy strip is 0.1% to 9%. In one or more embodiments detailed herein, a variation of the zinc weight percent between a surface and a thickness center of the aluminum alloy strip is 0.1% to 8%. In one or more embodiments detailed herein, a variation of the zinc weight percent between a surface and a thickness center of the aluminum alloy strip is 0.1% to 7%. In one or more embodiments detailed herein, a variation of the zinc weight percent between a surface and a thickness center of the aluminum alloy strip is 0.1% to 6%. In one or more embodiments detailed herein, a variation of the zinc weight percent between a surface and a thickness center of the aluminum alloy strip is 0.1% to 5%. In one or more embodiments detailed herein, a variation of the zinc weight percent is 0.1% to 4% between a surface and a thickness center of the aluminum alloy strip.

In one or more embodiments detailed herein, a variation of the zinc weight percent between a surface and a thickness center of the aluminum alloy strip is 1% to 15%. In one or more embodiments detailed herein, a variation of the zinc weight percent between a surface and a thickness center of the aluminum alloy strip is 2% to 15%. In one or more embodiments detailed herein, a variation of the zinc weight percent between a surface and a thickness center of the aluminum alloy strip is 3% to 15%. In one or more embodiments detailed herein, a variation of the zinc weight percent between a surface and a thickness center of the aluminum alloy strip is 4% to 15%. In one or more embodiments detailed herein, a variation of the zinc weight percent between a surface and a thickness center of the aluminum alloy strip is 5% to 15%. In one or more embodiments detailed herein, a variation of the zinc weight percent between a surface and a thickness center of the aluminum alloy strip is 6% to 15%. In one or more embodiments detailed herein, a variation of the zinc weight percent between a surface and a thickness center of the aluminum alloy strip is 7% to 15%. In one or more embodiments detailed herein, a variation of the zinc weight percent between a surface and a thickness center of the aluminum alloy strip is 8% to 15%. In one or more embodiments detailed herein, a variation of the zinc weight percent between a surface and a thickness center of the aluminum alloy strip is 9% to 15%. In one or more embodiments detailed herein, a variation of the zinc weight percent between a surface and a thickness center of the aluminum alloy strip is 10% to 15%. In one or more embodiments detailed herein, a variation of the zinc weight percent between a surface and a thickness center of the aluminum alloy strip is 11% to 15%. In one or more embodiments detailed herein, a variation of the zinc weight percent between a surface and a thickness center of the aluminum alloy strip is 12% to 15%.

In one or more embodiments detailed herein, the aluminum alloy has a zinc weight percent of 4% to 28% or any other weight percent range detailed herein and does not exhibit centerline segregation.

### Non-Limiting Method For Producing Aluminum Alloy Strip

In embodiments, the casting of the aluminum alloy strip detailed herein may be accomplished via a continuous casting apparatus capable of producing continuously cast products that are solidified at high solidification rates. One example of a continuous casting apparatus capable of achieving the above-described solidification rates is the apparatus described in U.S. Patent Nos. 6,672,368 and 7,125,612. In one or more embodiments detailed herein, the aluminum alloy strip is continuously cast using the Micromill^{™} process described in U.S. Patent Nos. 6,672,368 and 7,125,612.

In embodiments, as illustrated in Figures 1-2, a molten aluminum alloy metal M may be stored in a hopper H (or tundish) and delivered through a feed tip T, in a direction B, to a pair of rolls R₁ and R₂, having respective roll surfaces D₁ and D₂, which are each rotated in respective directions A₁ and A₂, to produce a solid cast product S. In one or more embodiments detailed herein, gaps G₁ and G₂ may be maintained between the feed tip T and respective rolls R₁ and R₂ as small as possible to prevent molten metal from leaking out, and to minimize the exposure of the molten metal to the atmosphere, while maintaining a separation between the feed tip T and rolls R₁ and R₂. A plane L through the centerline of the rolls R₁ and R₂ passes through a region of minimum clearance between the rolls R₁ and R₂ referred to as the roll nip N.

In one or more embodiments detailed herein, during casting, the molten metal M directly contacts the cooled rolls R₁ and R₂ at regions 2 and 4, respectively. Upon contact with the rolls R₁ and R₂, the metal M begins to cool and solidify. The cooling metal produces an upper shell 6 of solidified metal adjacent the roll R₁ and a lower shell 8 of solidified metal adjacent to the roll R₂. The thickness of the shells 6 and 8 increases as the metal M advances towards the nip N. Large dendrites 10 of solidified metal (not shown to scale) may be produced at the interfaces between each of the upper and lower shells 6 and 8 and the molten metal M. The large dendrites 10 may be broken and dragged into a center portion 12 of the slower moving flow of the molten metal M and may be carried in the direction of arrows C₁ and C₂. The dragging action of the flow can cause the large dendrites 10 to be broken further into smaller dendrites 14 (not shown to scale). In the central portion 12 upstream of the nip N referred to as a region 16, the metal M is semi-solid and may include a solid component (the solidified small dendrites 14) and a molten metal component. The metal M in the region 16 may have a mushy consistency due in part to the dispersion of the small dendrites 14 therein. At the location of the nip N, some of the molten metal may be squeezed backwards in a direction opposite to the arrows C₁ and C₂. The forward rotation of the rolls R₁ and R₂ at the nip N advances substantially only the solid portion of the metal (the upper and lower shells 6 and 8 and the small dendrites 14 in the central portion 12) while forcing molten metal in the central portion 12 upstream from the nip N such that the metal may be completely solid as it leaves the point of the nip N. In this manner and in one or more embodiments detailed herein, a freeze front of metal may be formed at the nip N. Downstream of the nip N, the central portion 12 may be a solid central portion, 18 containing the small dendrites 14 sandwiched between the upper shell 6 and the lower shell 8. In the central portion, 18, the small dendrites 14 may be 20 microns to 50 microns in size and have a generally globular shape. The three portions, of the upper and lower shells 6 and 8 and the solidified central portion 18, constitute a single, solid cast product (S in Figure 1 and element 20 in Figure 2). Thus, the aluminum alloy cast product 20 may include a first portion of an aluminum alloy and a second portion of the aluminum alloy (corresponding to the shells 6 and 8) with an intermediate portion (the solidified central portion18) therebetween. The solid central portion 18 may constitute 20 percent to 30 percent of the total thickness of the cast product 20.

The rolls R₁ and R₂ may serve as heat sinks for the heat of the molten metal M. In one embodiment, heat may be transferred from the molten metal M to the rolls R₁ and R₂ in a uniform manner to ensure uniformity in the surface of the cast product 20. Surfaces D₁ and D₂ of the respective rolls R₁ and R₂ may be made from steel, copper, nickel, or other suitable material and may be textured and may include surface irregularities (not shown) which may contact the molten metal M.

The control, maintenance and selection of the appropriate speed of the rolls R₁ and R₂ may impact the ability to continuously cast products. The roll speed determines the speed that the molten metal M advances towards the nip N. If the speed is too slow, the large dendrites 10 will not experience sufficient forces to become entrained in the central portion 12 and break into the small dendrites 14. In one or more embodiments detailed herein, the roll speed may be selected such that a freeze front, or point of complete solidification, of the molten metal M may form at the nip N. Accordingly, the present casting apparatus and methods may be suited for operation at high speeds such as those ranging from 7.6 to 152 m (25 to 500 feet) per minute; alternatively from 12.2 to 152 m (40 to 500 feet) per minute; alternatively from 12.2 to 122 m (40 to 400 feet) per minute; alternatively from 30.5 to 122 m (100 to 400 feet) per minute; and alternatively from 45.7 to 91.4 m (150 to 300 feet) per minute. The linear rate per unit area that molten aluminum is delivered to the rolls R₁ and R₂ may be less than the speed of the rolls R₁ and R₂ or about one quarter of the roll speed.

Continuous casting of aluminum alloys according to the present disclosure may be achieved by initially selecting the desired dimension of the nip N corresponding to the desired gauge of the cast product S. The speed of the rolls R₁ and R₂ may be increased to a desired production rate or to a speed which is less than the speed which causes the roll separating force increases to a level which indicates that rolling is occurring between the rolls R₁ and R₂. Casting at the rates contemplated by an embodiment of the present invention (i.e. 7.6 to 122 m (25 to 400 feet) per minute) solidifies the aluminum alloy cast product about 1000 times faster than aluminum alloy cast as an ingot cast and improves the properties of the cast product over aluminum alloys cast as an ingot. The rate at which the molten metal is cooled may be selected to achieve rapid solidification of the outer regions of the metal. Indeed, the cooling of the outer regions of metal may occur at a rate of at least 1000 degrees Celsius per second.

The continuous cast strip may be of any suitable thickness, and is generally of sheet gauge (0.152 mm to 6.32 mm (0.006 inch to 0.249 inch)) or thin-plate gauge (6.35 mm to 10.2 mm (0.250 inch to 0.400 inch)), i.e., has a thickness in the range of from 0.152 to 10.2 mm (0.006 inch to 0.400 inch). In one embodiment, the strip has a thickness of at least 1.02 mm (0.040 inch). In one embodiment, the strip has a thickness of less than 8.13 mm (0.320 inch).

### Macro-Segregation Procedure

Samples are first mounted and polished in Lucite using standard metallographic preparation techniques for aluminum. An Electron Probe Micro Analyzer ("EPMA") is used to profile the distribution of the alloying elements across a thickness to show the macro-segregation of the alloying elements.

EPMA line scans are set with an initial spot of 100 micrometers diameter about 50 micrometers from the sample surface moving in the thickness direction until the other surface is reached. The defocused beam spots are calculated to maintain a 50 micrometer separation to provide 50% overlap between points.

A JEOL JXA 8530F Field Emission Electron Probe Microanalyzer Hyperprobe with 4 Wave dispersive spectrometers and JEOL SDD-EDS are used to gather the data. The operating conditions are:
Accelerating Voltage: 15kV
Beam Intensity: 100nA
Defocus electron beam: 100µm
Line scan profile step 50 µm
Analyzed elements may include: Ti, Zr, Mg, Si, Mn, Fe, Cu, Zn and Al

The wave dispersive spectrometer (WDS) crystal and spectrometers are used as detailed in the Table 1.

**Table 1**

| Spectrometer | Diffracting Crystal | Counter | Element |
|---|---|---|---|
| 1 | PETJ | Gas Flow (P-10) | Ti, Zr |
| 2 | TAP | Gas Flow (P-10) | Mg, Si |
| 3 | LIFH | Sealed Xe gas | Mn, Fe |
| 4 | LIFL | Sealed Xe gas | Cu, Zn |
| 5 | | SDD-EDS | Al |

| | | | |
|---|---|---|---|
| The counting time is 10 seconds for all elements | | | |

A background measurement is collected every 50 spots for 5 seconds on positive and negative background locations. Elements measured are quantitatively analyzed using the JEOL quant ZAF analysis package for metals with atomic number correction by Philibert-Tixier method and flourescence excitation correction by Reed method.

Alternately, the concentration of alloying elements through depth of a sample was determined using a quantometer consistent with the method used to analyze the samples from U.S. Patent No. 6,672,368.

### Micro-Segregation Procedure

Samples are first mounted and polished in Lucite using standard metallographic preparation techniques for aluminum. An EPMA is used to profile the distribution of the alloying elements across a thickness to show the micro-segregation of the alloying elements.

EPMA line scans are set with a focused spot moving with a 1 micrometer step across several grains to provide overlapping points through multiple grains.

A JEOL JXA 8530F Field Emission Electron Probe Microanalyzer Hyperprobe with 4 Wave dispersive spectrometers and JEOL SDD-EDS are used to gather the data. The operating conditions are:
Accelerating Voltage: 15kV
Beam Intensity: 100nA
Focused electron beam
Line scan profile step 1 µm
Analyzed elements may include: Ti, Zr, Mg, Si, Mn, Fe, Cu, Zn and Al
The WDS crystal and spectrometers are used as detailed in Table 1.

A background measurement is collected every 50 spots for 5 seconds on positive and negative background locations. Elements measured are quantitatively analyzed using the JEOL quant ZAF analysis package for metals with atomic number correction by Philibert-Tixier method and flourescence excitation correction by Reed method.

### NON-LIMITING EXAMPLES

Aluminum alloy samples were cast using the apparatus detailed in U.S. Patent No. 6,672,368 at a speed of 16.8 m (55 feet) per minute to 25.9 m (85 feet) per minute and had a final thickness detailed in the tables below. The average weight percentages of the zinc, magnesium and copper from the surface to 3,000 micrometers thickness depth in each sample was determined using either the **"macro-segregation"** procedure detailed herein or via quantometer. Table 2 below shows the average weight percentages of zinc, copper and magnesium from surface to a thickness depth of 3,000 micrometers in each of the cast samples and the method used to determine the weight percentages in each sample:

**Table 2**

| Sample | Thickness (mm) | Avg. Zn wt.% | Avg. Mg wt.% | Avg. Cu wt.% | Method |
|---|---|---|---|---|---|
| 1 | 3.5 | 4.26 | 1.50 | 1.59 | macro-segregation procedure |
| 2 | 3.3 | 5.60 | 1.85 | 2.28 | quantometer |
| 3 | 3.9 | 6.38 | 1.47 | 1.53 | macro-segregation procedure |
| 4 | 3.4 | 7.34 | 2.13 | 1.90 | quantometer |
| 5 | 3.4 | 7.56 | 1.94 | 2.42 | quantometer |
| 6 | 4.1 | 8.71 | 1.68 | 1.43 | macro-segregation procedure |
| 7 | 3.9 | 15.98 | 1.21 | 1.53 | macro-segregation procedure |
| 8 | 3.6 | 27.46 | 0.97 | 1.64 | macro-segregation procedure |

Table 3 below shows the variation of zinc weight percentages in each of the samples from surface to a thickness depth of 3,000 micrometers:

**Table 3**

| Sample | Min. Zn wt.% | Max. Zn wt.% | Avg. Zn wt.% | Variation (%) |
|---|---|---|---|---|
| 1 | 3.91 | 4.52 | 4.26 | 14.40 |
| 2 | 5.40 | 5.75 | 5.60 | 6.25 |
| 3 | 6.17 | 6.66 | 6.38 | 7.68 |
| 4 | 7.11 | 7.54 | 7.34 | 5.86 |
| 5 | 6.95 | 7.71 | 7.56 | 10.05 |
| 6 | 8.34 | 8.96 | 8.71 | 7.12 |
| 7 | 15.10 | 17.09 | 15.98 | 12.45 |
| 8 | 25.53 | 29.70 | 27.46 | 15.19 |

The average weight percentages of the zinc, magnesium and copper from the surface to the thickness center in each sample were determined using either the **"macro-segregation"** procedure detailed herein or via quantometer. Table 4 below shows the average weight percentages of zinc, copper and magnesium from surface to a thickness center in each of the cast samples and the method used to determine the weight percentages in each sample:

**Table 4**

| Sample | Thickness (mm) | Avg. Zn wt.% | Avg. Mg wt.% | Avg. Cu wt.% | Method |
|---|---|---|---|---|---|
| 1 | 3.5 | 4.27 | 1.50 | 1.61 | macro-segregation procedure |
| 2 | 3.3 | 5.64 | 1.86 | 2.28 | quantometer |
| 3 | 3.9 | 6.36 | 1.47 | 1.52 | macro-segregation procedure |
| 4 | 3.4 | 7.33 | 2.12 | 1.88 | quantometer |
| 5 | 3.4 | 7.54 | 1.93 | 2.42 | quantometer |
| 6 | 4.1 | 8.71 | 1.70 | 1.42 | macro-segregation procedure |
| 7 | 3.9 | 15.97 | 1.21 | 1.52 | macro-segregation procedure |
| 8 | 3.6 | 27.54 | 0.99 | 1.70 | macro-segregation procedure |

Table 5 below shows the variation of zinc weight percentages in each of the samples from surface to a thickness center in each sample:

**Table 5**

| Sample | Min. Zn wt.% | Max. Zn wt.% | Avg. Zn wt.% | Variation (%) |
|---|---|---|---|---|
| 1 | 3.91 | 4.52 | 4.27 | 14.29 |
| 2 | 5.48 | 5.75 | 5.64 | 4.79 |
| 3 | 6.17 | 6.57 | 6.36 | 6.29 |
| 4 | 7.11 | 7.54 | 7.33 | 5.87 |
| 5 | 6.95 | 7.71 | 7.54 | 10.08 |
| 6 | 8.44 | 8.96 | 8.71 | 5.97 |
| 7 | 15.10 | 17.09 | 15.97 | 12.46 |
| 8 | 25.96 | 29.70 | 27.54 | 13.58 |

The data generated for each sample is plotted in Figures 3-10. A comparison the weight percentages of the zinc, magnesium and copper through thickness of a direct chill cast prior art product and a continuously cast prior art product of U.S. Patent No. 6,672,368 are also included as Figures 11-12 for comparison.

As shown in Figures 3-10 and the tables above, the inventors surprisingly found that the variation of the zinc weight percent between a surface and a thickness depth of 3,000 micrometers in samples 1-7 is less than 15%. Moreover, the variation of the zinc weight percent between a surface and a thickness depth of 3,000 micrometers of sample 8 is greater than 15%. Similarly, based on visual inspection of Figures 11-12, the variation of the zinc weight percent between a surface and a thickness depth of 3,000 micrometers in the direct chill cast prior art product and the continuously cast prior art product is greater than 15%.

As shown in Figures 3-10 and the tables above, the inventors surprisingly found that the variation of the zinc weight percent between a surface and a thickness center in samples 1-8 according to the present invention is less than 15%. Moreover, based on visual inspection of Figures 11-12, the variation of the zinc weight percent between a surface and a thickness center of the direct chill cast prior art product and the continuously cast prior art product is greater than 15%.

The weight percentages of the zinc, magnesium and copper across grains from the surface to 200 micrometers thickness depth in sample 6 was determined using the "micro-segregation" procedure detailed herein. The data is presented in Figure 13. For comparison, the weight percentages of the zinc, magnesium and copper across grains through thickness for a direct chill cast prior art product are shown in Figure 14. As shown in Figure 13, the inventors surprisingly found that the weight percent of the primary alloying elements Zn, Cu and Mg were substantially uniform across the grains within the matrix with an increase in the weight percent of the alloying elements at the positions of second phase particles at grain boundaries and within the grains.

Figure 15 shows the structure of sample 6. The structure of samples of aluminum alloys having average zinc contents of 16% and 25% cast using the apparatus detailed in U.S. Patent No. 6,672,368 at a speed of 16.8 m (55 feet) per minute are shown in Figures 16 and 17, respectively. Figures 15-17 show products of the present invention have a globular grain structure and are substantially free of micro-segregation. Moreover, as illustrated in Figures 15-17, the products of the present invention may be substantially free of dendrites and consist primarily of globular non-dendritic grains - i.e., a globular grain structure. Also, as shown by the absence of shading within the grains of Figures 15-17 when the samples are observed in polarized light, the products are substantially free of micro-segregation effects.

While a number of embodiments of the present invention have been described, it is understood that these embodiments are illustrative only, and not restrictive, and that many modifications, within the scope of the claims, may become apparent to those of ordinary skill in the art. Further still, the various steps may be carried out in any desired order (and any desired steps may be added and/or any desired steps may be eliminated).

## Claims

1. A cast product comprising:
an aluminum alloy strip;
wherein the aluminum alloy strip comprises:
4 wt. % to 28 wt. % zinc;
optionally at least one of 1 wt. % to 3 wt. % Cu and 1 wt. % to 3 wt. % Mg;
optionally 0.1 wt. % to 1.0 wt. % Mn;
optionally 0.05 wt. % to 0.3 wt. % Cr;
optionally 0.04 wt. % to 0.25 wt. % Zr;
the balance being aluminum and impurities,
wherein the aluminum alloy strip has a thickness (T),
wherein the aluminum alloy realizes a zinc variation of not greater than 15% as measured between a surface (S) of the aluminum alloy strip and a center (T/2) of the aluminum alloy strip,
wherein the zinc variation is calculated as {(the maximum weight percent of zinc from the surface (S) to the thickness center (T/2) minus (-) the minimum weight percent of zinc from the surface (S) to the thickness center (T/2)) divided by (/) (the mean weight percent of the zinc from the surface (S) to the thickness center (T/2))}*100, wherein the weight percent of zinc is measured according to the macro-segregation procedure disclosed in the description.

2. The cast product of claim 1, wherein the aluminum alloy strip comprises 6 wt. % to 28 wt. % zinc.

3. The cast product of claim 1, wherein the aluminum alloy strip comprises 8 wt. % to 28 wt. % zinc.

4. The cast product of claim 1, wherein the aluminum alloy strip comprises 10 wt. % to 28 wt. % zinc.

5. The cast product of claim 1, wherein the aluminum alloy strip comprises 4 wt. % to 15 wt. % zinc

6. The cast product of claim 1, wherein the aluminum alloy strip comprises 6 wt. % to 12 wt. % zinc.

7. The cast product of claim 1, wherein the aluminum alloy strip comprises 4 wt. % to 10 wt. % zinc.

8. The cast product of claim 1, wherein the aluminum alloy strip comprises 4 wt. % to 8 wt. % zinc.

9. The cast product of claim 1, wherein the aluminum alloy strip comprises 4 wt. % to 12 wt. % zinc.

10. The cast product of any of claims 1-9, wherein the aluminum alloy strip comprises 1 wt. % to 2.5 wt. % copper, or 1 wt. % to 2.0 wt. % copper, or 1 wt. % to 1.5 wt. % copper.

11. The cast product of any of claims claims 1-10, wherein the aluminum alloy strip comprises 1 wt. % to 2.5 wt. % magnesium, or 1 wt. % to 2.0 wt. % magnesium, or 1 wt. % to 1.5 wt. % magnesium.

12. The cast product of any of the preceding claims, wherein the zinc variation is not greater than 12%, or wherein the zinc variation is not greater that 10 %, or wherein the zinc variation is not greater that 8 %, or wherein the zinc variation is not greater than 6 %, or wherein the zinc variation is not greater than 5 %.

## Patentansprüche

1. Gießprodukt, umfassend:
ein Aluminiumlegierungsband;
wobei das Aluminiumlegierungsband Folgendes umfasst:
4 Gew.-% bis 28 Gew.-% Zink;
optional mindestens eines aus 1 Gew.-% bis 3 Gew.-%. Cu und 1 Gew.-% bis 3 Gew.-% Mg;
optional 0,1 Gew.-% bis 1,0 Gew.-% Mn;
optional 0,05 Gew.-% bis 0,3 Gew.-% Cr;
optional 0,04 Gew.-% bis 0,25 Gew.-% Zr;
wobei der Rest Aluminium und Verunreinigungen ist,
wobei das Aluminiumlegierungsband eine Dicke (T) aufweist,
wobei die Aluminiumlegierung eine Zinkvariation von nicht mehr als 15 %, gemessen zwischen einer Oberfläche (S) des Aluminiumlegierungsbandes und einem Zentrum (T/2) des Aluminiumlegierungsbandes, realisiert,
wobei die Zinkvariation berechnet wird als {(maximaler Gewichtsprozentsatz von Zink von der Oberfläche (S) bis zu dem Dickenzentrum (T/2) minus (-) minimaler Gewichtsprozentsatz von Zink von der Oberfläche (S) bis zu dem Dickenzentrum (T/2)) geteilt durch (/) (mittlerer Gewichtsprozentsatz von Zink von der Oberfläche (S) bis zu dem Dickenzentrum (T/2))}*100, wobei der Gewichtsprozentsatz von Zink gemäß dem in der Beschreibung offenbarten Makrosegregationsverfahren gemessen wird.

2. Gießprodukt nach Anspruch 1, wobei das Aluminiumlegierungsband 6 Gew.-% bis 28 Gew.-% Zink umfasst.

3. Gießprodukt nach Anspruch 1, wobei das Aluminiumlegierungsband 8 Gew.-% bis 28 Gew.-% Zink umfasst.

4. Gießprodukt nach Anspruch 1, wobei das Aluminiumlegierungsband 10 Gew.-% bis 28 Gew.-% Zink umfasst.

5. Gießprodukt nach Anspruch 1, wobei das Aluminiumlegierungsband 4 Gew.-% bis 15 Gew.-% Zink umfasst.

6. Gießprodukt nach Anspruch 1, wobei das Aluminiumlegierungsband 6 Gew.-% bis 12 Gew.-% Zink umfasst.

7. Gießprodukt nach Anspruch 1, wobei das Aluminiumlegierungsband 4 Gew.-% bis 10 Gew.-% Zink umfasst.

8. Gießprodukt nach Anspruch 1, wobei das Aluminiumlegierungsband 4 Gew.-% bis 8 Gew.-% Zink umfasst.

9. Gießprodukt nach Anspruch 1, wobei das Aluminiumlegierungsband 4 Gew.-% bis 12 Gew.-% Zink umfasst.

10. Gießprodukt nach einem der Ansprüche 1-9, wobei das Aluminiumlegierungsband 1 Gew.-% bis 2,5 Gew.-% Kupfer oder 1 Gew.-% bis 2,0 Gew.-% Kupfer oder 1 Gew.-% bis 1,5 Gew.-% Kupfer umfasst.

11. Gießprodukt nach einem der Ansprüche 1-10, wobei das Aluminiumlegierungsband 1 Gew.-% bis 2,5 Gew.-% Magnesium oder 1 Gew.-% bis 2,0 Gew.-% Magnesium oder 1 Gew.-% bis 1,5 Gew.-% Magnesium umfasst.

12. Gießprodukt nach einem der vorhergehenden Ansprüche, wobei die Zinkvariation nicht größer als 12 % ist oder wobei die Zinkvariation nicht größer als 10 % ist oder wobei die Zinkvariation nicht größer als 8 % ist, oder wobei die Zinkvariation nicht größer als 6 % ist oder wobei die Zinkvariation nicht größer als 5 % ist.

## Revendications

1. Produit coulé comprenant :
une bande d'alliage d'aluminium ;
dans lequel la bande d'alliage d'aluminium comprend :
4 % en poids à 28 % en poids de zinc ;
éventuellement au moins 1 % en poids à 3 % en poids de Cu et 1 % en poids à 3 % en poids de Mg ;
éventuellement 0,1 % en poids à 1,0 % en poids de Mn ;
éventuellement 0,05 % en poids à 0,3 % en poids de Cr ;
éventuellement 0,04 % en poids à 0,25 % en poids de Zr ;
le reste étant constitué d'aluminium et d'impuretés,
dans lequel la bande d'alliage d'aluminium a une épaisseur (T) ,
dans lequel l'alliage d'aluminium réalise une variation de zinc non supérieure à 15 % telle que mesurée entre une surface (S) de la bande d'alliage d'aluminium et un centre (T/2) de la bande d'alliage d'aluminium ,
dans lequel la variation de zinc est calculée comme étant {(le pourcentage en poids maximum de zinc de la surface (S) au centre d'épaisseur (T/2) moins (-) le pourcentage en poids minimum de zinc de la surface (S) au centre d'épaisseur (T/2)) divisé par (/) (le pourcentage en poids moyen du zinc de la surface (S) au centre d'épaisseur (T/2))}*100, le pourcentage en poids de zinc étant mesuré selon la procédure de macroségrégation divulguée dans l'invention.

2. Produit coulé selon la revendication 1, dans lequel la bande d'alliage d'aluminium comprend 6 % en poids à 28 % en poids de zinc.

3. Produit coulé selon la revendication 1, dans lequel la bande d'alliage d'aluminium comprend 8 % en poids à 28 % en poids de zinc.

4. Produit coulé selon la revendication 1, dans lequel la bande d'alliage d'aluminium comprend 10 % en poids à 28 % en poids de zinc.

5. Produit coulé selon la revendication 1, dans lequel la bande d'alliage d'aluminium comprend 4 % en poids à 15 % en poids de zinc

6. Produit coulé selon la revendication 1, dans lequel la bande d'alliage d'aluminium comprend 6 % en poids à 12 % en poids de zinc.

7. Produit coulé selon la revendication 1, dans lequel la bande d'alliage d'aluminium comprend 4 % en poids à 10 % en poids de zinc.

8. Produit coulé selon la revendication 1, dans lequel la bande d'alliage d'aluminium comprend 4 % en poids à 8 % en poids de zinc.

9. Produit coulé selon la revendication 1, dans lequel la bande d'alliage d'aluminium comprend 4 % en poids à 12 % en poids de zinc.

10. Produit coulé selon l'une quelconque des revendications 1 à 9, dans lequel la bande d'alliage d'aluminium comprend 1 % en poids à 2,5 % en poids de cuivre, ou 1 % en poids à 2,0 % en poids de cuivre, ou 1 % en poids à 1,5 % en poids de cuivre.

11. Produit coulé selon l'une quelconque des revendications 1 à 10, dans lequel la bande d'alliage d'aluminium comprend 1 % en poids à 2,5 % en poids de magnésium, ou 1 % en poids à 2,0 % en poids de magnésium, ou 1 % en poids à 1,5 % en poids de magnésium.

12. Produit coulé selon l'une quelconque des revendications précédentes, dans lequel la variation de zinc n'est pas supérieure à 12 %, ou dans lequel la variation de zinc n'est pas supérieure à 10 %, ou dans lequel la variation de zinc n'est pas supérieure à 8 %, ou dans lequel la variation de zinc n'est pas supérieure à 6 %, ou dans lequel la variation de zinc n'est pas supérieure à 5 %.
